

Dec. 12, 1950

G. H. KEYES ET AL

2,533,472

UNSYMMETRICAL OXONOL FILTER AND ANTIHALATION DYES

Filed Jan. 17, 1947

Fig. 1



Fig. 2



Fig. 3



Grafton H. Keyes  
Leslie G. S. Brooker  
INVENTORS

By *Norman M. Perrier*  
*R. Frank Smith*  
ATTORNEYS

## UNITED STATES PATENT OFFICE

2,533,472

UNSYMMETRICAL OXONOL FILTER AND  
ANTIHALATION DYES

Grafton H. Keyes and Leslie G. S. Brooker, Rochester, N. Y., assignors to Eastman Kodak Company, Rochester, N. Y., a corporation of New Jersey

Application January 17, 1947, Serial No. 722,740

5 Claims. (Cl. 95—2)

1

This invention relates to improvements in photographic elements and more particularly in photographic elements having light screening substances therein.

It is known that photographic elements require, for many purposes, to have light screening substances incorporated therein. Such a light screening substance may be in a layer overlying a light sensitive emulsion or overlying two or more light sensitive emulsions; or it may be in a light sensitive emulsion for the purpose of modifying a light record in such emulsion or of protecting an underlying light sensitive emulsion or emulsions from the action of light of wavelength absorbed by such light screening substance; or it may be in a layer not containing a light sensitive substance but arranged between two light sensitive emulsions; or it may be in a layer serving as a backing on an element having one or more light sensitive emulsions (for example, to reduce halation).

In particular, light screening substances are often required (a) in overcoatings upon photographic elements to protect the light sensitive emulsion or emulsions from the action of light which it is not desired to record, e. g. ultraviolet light in the case of still or moving pictures, especially color pictures, (b) in layers arranged between differentially color-sensitized emulsions, e. g. to protect red- and green-sensitized emulsions from the action of blue light and (c) in backings, forming the so-called anti-halation layers, on either side of a transparent support carrying the light-sensitive emulsion or emulsions.

In most cases, and especially when the element contains a color-sensitized emulsion or color-sensitized emulsions, it is particularly desirable to employ light-screening substances which do not affect the general sensitivity or the color sensitivity of light-sensitive emulsions with which they may come into contact. It is also particularly desirable to employ light-screening substances which do not substantially diffuse from the layers or coatings in which they are incorporated, either during the manufacture of the element or on keeping it or in photographically processing it. Finally, it is generally necessary to employ light-screening substances which can readily be rendered ineffective, i. e. decolorized or destroyed and removed, prior to or during or after photographic processing; for many purposes it is particularly convenient to employ light-screening substances which are rendered ineffective by one of the photographic baths employed in proc-

2

essing the element after exposure, e. g. a photographic developing bath or fixing bath or a silver-oxidizing (including silver-removing) bath. For example, in an element which is to be processed by reversal, it is often convenient to employ a light-screening substance which is rendered ineffective by the developer employed to develop the latent image or images to silver since exposure to light of the residual light sensitive emulsion or emulsions may thereby be facilitated. This is particularly the case when, in making color photographs, several differentially color-sensitized emulsions, constituted, for example, by silver halide, such as silver bromide dispersed in gelatin, collodion or other colloid, are coated on one or both sides of a support, for example in inseparably-superimposed layers. Such differentially color-sensitized emulsions have to be processed to different colors and to facilitate the differential color-processing, methods involving selective exposure of light sensitive images in the layers may be employed. Such selective re-exposure, e. g. of silver halide remaining undeveloped in development of the latent images formed in silver halide emulsion layers (residual silver halide) is often facilitated if the light-screening substance which was present during the original exposure is decolorized or removed in the developing bath employed to develop the latent images to silver. Any of the elements referred to above may be such that one or more of the emulsions contain coupling components, e. g. those described in French Patent 834,371, granted August 16, 1938.

35 Numerous substances have been employed as light-screening substances for the purposes indicated above. Many of these are known yellow dyes but it has proved extremely difficult to find dyes having the combination of qualities desired.

40 Many are not resistant to diffusion and wander rather freely from the layer in which it is intended that they should remain; many adversely affect the sensitivity of light sensitive emulsions with which they come into contact (a number of these reduce the general sensitivity or some specific color sensitivity thereof, but others of them may even impart an additional and unwanted specific color sensitivity thereto).

45 We have now found a class of dyes which satisfactorily fulfill the requirements of filter and antihalation dyes for use in photographic elements. This class consists of certain unsymmetrical methineoxonol and polymethineoxonol dyes. These dyes are characterized by the fact that they contain the oxochromic atoms O= and

—OH connected by a conjugating chain of carbon atoms. We propose to use dyes in which one end of the conjugated carbon chain is connected to a barbituric acid, thiobarbituric acid, pyrazolone, oxindole, indandione or isoxazolone ring and the opposite end of the chain is connected to a cyanoacetyl benzofuran or benzoyl acetonitrile group.

In the drawing, the figures are enlarged sectional views of photographic elements showing overcoating filter and anti-halation layers according to our invention.

The compounds which we propose to use as screening dyes have the following general formula:



OR



where X represents the atoms necessary to complete a barbituric acid, thiobarbituric acid, pyrazolone, oxindole, indandione or isoxazolone ring, Y is an aryl nucleus of the benzene series or a benzofuran group and n is 0, 1 or 2.

The general formula indicates that our compound may be depicted in two electromeric forms.

The following examples illustrate compounds which may be used according to our invention.

**EXAMPLE 1**



[2,4-dimethylbenzoylacetonitrile]-[3-methyl-1-phenyl-5-pyrazolone-(4)] trimethineoxonol

3.45 g. (1 mol.) of 4-(3-acetanilidoallylidene)-3-methyl-1-phenyl-5-pyrazolone, 1.7 g. (1 mol.) of 2,4-dimethylbenzoylacetone, 20 cc. of pyridine and 1 g. (1 mol.) of triethylamine were refluxed for 15 minutes. The reaction mixture was chilled and then acidified with hydrochloric acid. A tarry mass separated. After decantation of liquors the somewhat tarry residue was stirred up in presence of a small amount of methyl alcohol and soon became crystalline. It was collected on filter, washed with methyl alcohol and dried. It was purified by dissolving in methyl alcohol as the triethylamine salt, filtering hot, acidifying and chilling. After two such treatments the dye was obtained as brownish orange crystals, M. P. 139-141° with decomposition. The pinkish orange solution of the triethylamine salt was bleached by developer.

**EXAMPLE 2**



3.8 g. (1 mol.) of 2-(5-acetanilido-2,4-pentadienylidene cyanoacetyl) benzofuran, 1.85 g. (1

and 1 g. (1 mol.) of triethylamine were heated together at the temperature of a steam bath for 10 minutes. The mixture was then chilled and made acidic with dilute hydrochloric acid. The dye which separated was collected on filter, washed with methyl alcohol and dried. It was purified by dissolving as the triethylamine salt, filtering hot and then acidifying and chilling. Two such treatments gave the dye as a dark purplish solid, M. P. 195-197° with decomposition. The blue solution of the triethylamine salt was bleached by developer.

15 was bleached by development.

The 2-(5-acetanilido-2,4-pentadienylidine cyanoacetylbenzofuran employed in the above preparation was made by refluxing a mixture of 3.7 g. (1 mol.) of 2-cyanoacetylbenzofuran, 5.5 g. (1 mol.) of glutaconic aldehyde dianilide hydrochloride, 25 cc. of acetic anhydride and 1.65 g. (1 mol.) of fused sodium acetate for 2 to 3 minutes. The product separated on chilling, it was collected on filter, washed with water and methyl alcohol and used without further purification.

**EXAMPLE 3**



[2-cyanoacetylbenzofuran]-[3-methyl-1-p-sulfo-phenyl-5-pyrazolone-(4)] trimethineoxonol

35 1.7 g. (1 mol.) of 2-(3-acetanilidoallylideneaceto-  
anoacetyl) benzofuran, 1.3 g. (1 mol.) of 3-  
methyl-1-p-sulfophenyl-5-pyrazolone, 20 cc. of  
pyridine and 1 g. (2 mol.) of triethylamine were  
mixed together and heated on steam bath for 15  
minutes. Dye separated from the chilled re-  
40 action mixture on treatment with excess of dilute  
hydrochloric acid. The crude, washed dye was  
purified by dissolving the dye in hot alcohol as  
the triethylamine salt, filtering hot and precipi-  
tating from the chilled filtrate on acidification.  
45 Two such treatments gave the dye as a brownish  
crystalline powder M. P. 240-242° C. dec. Its  
bluish red solution of the triethylamine salt was  
readily bleached by developer.

The 2-(3-acetanilidoallylidene cyanoacetyl) benzofuran employed in the above was made by refluxing a mixture of 3 g. (1 mol.) of 2-cyanoacetylbenzofuran, 5.2 g. (1 mol.) of  $\beta$ -anilinoacrolein anil hydrochloride, 20 cc. of acetic anhydride and 2 g. (1 mol.) of triethylamine for 15 minutes. The product separated on chilling and was collected, washed on the filter and used without further purification.

**EXAMPLE 4**



[2-cyanoacetylbenzofuran]-[3-methyl-1-phenyl-5-pyrazolone-(4)] methineoxonol

3.2 g. (1 mol.) of 4-acetanilidomethylene-3-methyl-1-phenyl-5-pyrazolone, 1.85 g. (1 mol.) of 2-cyanoacetylbenzofuran, 30 cc. of absolute ethyl alcohol and 2 g. (2 mol.) of triethylamine were refluxed together for a period of one hour. Dye was separated from the chilled reaction mixture on acidification. Crude, washed dye was purified by

recrystallization as the triethylamine salt and precipitation with acid. The dye was obtained as yellow crystals, M. P. 141-143° C. with decomposition. Its solution is yellow.

## EXAMPLE 5



[2-cyanoacetylbenzofuran]-[1,3-diphenylbarbituric acid-(5)] trimethineoxonol

4.1 g. (1 mol.) of 5-(3-acetanilidoallylidine)-1,3-diphenyl barbituric acid, 1.8 g. (1 mol.) of 2-cyanoacetylbenzofuran, 40 cc. of pyridine and

## [2-cyanoacetylbenzofuran]-[1,3-diethyl-2-thiobarbituric acid-(5)] pentamethineoxonol

2 g. (1 mol.) of 5-(5-acetanilido-2,4-pentadienylidene)-1,3-diethyl-2-thiobarbituric acid, 0.9 g. (1 mol.) of 2-cyanoacetylbenzofuran, 20 cc. of pyridine and 1 g. (2 mol.) of triethylamine were mixed together and stood at room temperature for 15 minutes. Dye separated from this reaction mixture on chilling and acidification with dilute hydrochloric acid. The crude, washed dye was purified by dissolving in methyl alcohol as the triethylamine salt, filtering hot and precipitating from the chilled filtrate on acidification. Two such treatments gave the dye as a very dark solid M. P. 185-187° C., with decomposition. The solution of the triethylamine salt was bluish red, readily bleached.

## EXAMPLE 8



[2-cyanoacetyl-5-phenylbenzofuran]-[1,3-di-p-phenethylbarbituric acid-(5)] pentamethineoxonol

2 g. (2 mol.) of triethylamine were heated together under reflux for 10 minutes. Dye separated from the chilled reaction mixture on acidification with dilute hydrochloric acid. The crude, washed dye was purified by recrystallization as the triethylamine salt and precipitation on acidification. It was obtained as brownish crystals, M. P. 224°-226° C., with decomposition.

It give a bluish red solution in alcohol and triethylamine and was bleached readily by developer.

The 5-(3-acetanilidoallylidine)-1,3-diphenylbarbituric acid employed above was made by refluxing together equimolecular portions of 1,3-diphenylbarbituric acid,  $\beta$ -anilino acrolein anil hydrochloride and triethylamine in the presence of acetic anhydride for 30 minutes. The product separated on chilling and was collected, washed on filter and used without further purification.

## EXAMPLE 6



[2-cyanoacetylbenzofuran]-[3-methyl-1-phenyl-5-pyrazolone-(4)] trimethineoxonol

3.45 g. (1 mol.) of 4-(3-acetanilidoallylidine)-3-methyl-1-phenyl-5-pyrazolone, 1.85 g. (1 mol.) of 2-cyanoacetylbenzofuran, 20 cc. of pyridine and 1 g. (1 mol.) of triethylamine were refluxed together for ten minutes. Dye separated from the chilled reaction mixture on treatment with excess of dilute hydrochloric acid. The crude washed dye was purified by dissolving in alcohol as the triethylamine salt, filtering hot and precipitating from the chilled filtrate on acidification. Two such treatments gave the dye as very dark, purplish crystals, M. P. 242°-244° C., with decomposition.

## EXAMPLE 7



5 (1 mol.) of 2-cyanoacetylbenzofuran, 20 cc. of pyridine and 1 g. (2 mol.) of triethylamine were mixed together and stood at room temperature for 15 minutes. Dye separated from this reaction mixture on chilling and acidification with dilute hydrochloric acid. The crude, washed dye was purified by dissolving in methyl alcohol as the triethylamine salt, filtering hot and precipitating from the chilled filtrate on acidification. Two such treatments gave the dye as a very dark solid M. P. 185-187° C., with decomposition. The solution of the triethylamine salt was bluish red, readily bleached.

## EXAMPLE 8



[2-cyanoacetyl-5-phenylbenzofuran]-[1,3-di-p-phenethylbarbituric acid-(5)] pentamethineoxonol

30 5.6 g. (1 mol.) of 5-(5-acetanilido-2,4-pentadienylidene) 1,3-p-phenethylbarbituric acid, 2.6 g. (1 mol.) of 2-cyanoacetyl-5-phenylbenzofuran, 25 cc. of pyridine and 1 g. (1 mol.) of triethylamine were mixed together and heated at steam bath temperature for 10 minutes. Dye separated from the chilled reaction mixture on acidification with dilute hydrochloric acid. The crude, washed dye was purified in the usual manner and obtained as a blackish-brown powder, M. P. 175-177° C., with decomposition. The solution was blue.

The 5-(5-acetanilido-2,4-pentadienylidene)-1,3-p-phenethylbarbituric acid employed above was made heating together under reflux a mixture of equimolecular portions of 1,3-di-p-phenethyl barbituric acid, glutaconic aldehyde di-anilide hydrochloride, sodium acetate in acetic anhydride. The product separated on chilling and was collected, washed on filter and used without further purification. The 2-cyanoacetyl-5-phenylbenzofuran employed above was made in a manner similar to that described by Burger and Dienet, J. A. C. S. 67, 569 (1945) in making a cyanoacetylbenzofuran.

55 3.45 g. (1 mol.) of 4-(3-acetanilidoallylidine)-3-methyl-1-phenyl-5-pyrazolone, 1.85 g. (1 mol.) of 2-cyanoacetylbenzofuran, 20 cc. of pyridine and 1 g. (1 mol.) of triethylamine were refluxed together for ten minutes. Dye separated from the chilled reaction mixture on treatment with excess of dilute hydrochloric acid. The crude washed dye was purified by dissolving in alcohol as the triethylamine salt, filtering hot and precipitating from the chilled filtrate on acidification. Two such treatments gave the dye as very dark, purplish crystals, M. P. 242°-244° C., with decomposition.

## EXAMPLE 9



[Benzoylacetetonitrile]-[1,3-diethyl-2-triobarbituric acid-(5)] pentamethineoxonol

65 2 g. (1 mol.) of 5-(5-acetanilido-2,4-pentadienylidene)-1,3-diethyl-2-thiobarbituric acid, 0.7 g. (1 mol.) of benzoylacetetonitrile, 20 cc. of pyridine and 1 g. (2 mol.) of triethylamine were mixed together and stood at room temperature for 15 minutes. Dye separated from this reaction mixture on chilling and acidification with dilute hydrochloric acid. The crude, washed dye was purified in the usual way and obtained as very dark crystals, M. P. 164-166° C., with decomposition. The solution of the triethylamine salt was purple, readily bleached.

7  
EXAMPLE 10

[2-cyanoacetylbenzofuran]-[1-ethyloxindole-(3)-1-pentamethineoxonol

3.8 g. (1 mol.) of 2-(5-acetanilido-2,4-penta-dienylidine cyanoacetyl) benzofuran, 3.7 g. (1 mol.) of 1,3-di-p-phenetylbarbituric acid, 20 cc. of pyridine and 1 g. (1 mol.) of triethylamine were mixed together and heated at steam bath temperature for 15 minutes. Dye separated from the reaction mixture on chilling and acidification with dilute hydrochloric acid. The crude, washed dye was purified in the usual manner. It was obtained as very dark crystals. M. P. 192-194° C., with decomposition. The solution was blue.

10

## 8

[2-cyanoacetylbenzofuran]-[1,3-di-p-phenetylbarbituric acid-(5)-1-pentamethineoxonol

3.8 g. (1 mol.) of 2-(5-acetanilido-2,4-penta-dienylidine cyanoacetyl) benzofuran, 3.7 g. (1 mol.) of 1,3-di-p-phenetylbarbituric acid, 20 cc. of pyridine and 1 g. (1 mol.) of triethylamine were mixed together and heated at steam bath temperature for 15 minutes. Dye separated from the reaction mixture on chilling and acidification with dilute hydrochloric acid. The crude, washed dye was purified in the usual manner. It was obtained as very dark crystals. M. P. 192-194° C., with decomposition. The solution was blue.

10

## EXAMPLE 13



[3-carboxymethyl-1-phenyl-5-pyrazolone-(4)-2-cyanoacetylbenzofuran] pentamethineoxonol

25

3.8 g. (1 mol.) of 2-(5-acetanilido-2,4-penta-dienylidine cyanoacetyl) benzofuran, 2.2 (1 mol.) of 3-carboxymethyl-1-phenyl-5-pyrazolone, 20 cc. of pyridine and 1 g. (1 mol.) of triethylamine were refluxed together for 10 minutes. Dye separated from the chilled reaction mixture on acidification with dilute hydrochloric acid. The crude, washed dye was purified in the usual manner and obtained as a dark brown felt. M. P. 189-191° C., with decomposition. The solution was blue.

30

35

## EXAMPLE 11



[2-cyanoacetylbenzofuran]-[1,3-di-β-methoxyethylbarbituric acid-(5)-1-pentamethineoxonol

4.4 g. (1 mol.) of 5-(5-acetanilido-2,4-penta-dienylidine)-1,3-di-β-methoxyethylbarbituric acid, 1.85 g. (1 mol.) of 2-cyanoacetylbenzofuran, 20 cc. of pyridine and 1 g. (1 mol.) of triethylamine were mixed together and heated at steam bath temperature for ten minutes. Dye separated from the reaction mixture on chilling and acidification with dilute hydrochloric acid. The crude, washed dye was purified in the usual manner. It was obtained as purplish brown powder, M. P. 166-168° C., with decomposition.

The 5-(5-acetanilido-2,4-pentadienylidine)-1,3-di-β-methoxyethylbarbituric acid employed above was made by refluxing a mixture of equimolecular portions of 1,3-di-β-methoxyethylbarbituric acid, glutaconic aldehyde dianilide hydrochloride, fused sodium acetate in acetic anhydride for 2 to 3 minutes. The product separated on chilling, collected and washed on filter and used without further purification.

The 1,3-di(β-methoxyethyl) barbituric acid employed above was made according to the method used by Whitely J. C. S. 91, 1338 (1907) in preparing 1,3-diphenylbarbituric acid. The 1,3-di(β-methoxyethyl) barbituric acid was obtained as colorless crystals melting at 59-60°

40

## EXAMPLE 14



[2-cyanoacetylbenzofuran]-[3-methyl-1-p-tolyl-5-pyrazolone-(4)-1-methineoxonol

45

50

55

3.3 g. (1 mol.) of 2-acetanilidomethylene cyanoacetylbenzofuran, 2 g. (1 mol.) of 3-methyl-1-p-tolyl-5-pyrazolone, 25 cc. of pyridine, and 1 g. (1 mol.) of triethylamine were refluxed together for ten minutes. Dye separated from the chilled reaction mixture on acidification with dilute hydrochloric acid. The crude, washed dye was purified in the usual manner. It was obtained as buff powder, M. P. 243-245° C., with decomposition. The solution of its triethylamine salt was yellow.

60

## EXAMPLE 15



## EXAMPLE 12



## [2-cyanoacetylbenzofuran] [1,3-indandione-(2)] pentamethineoxonol

3.8 g. (1 mol.) of 2-(5-acetanilido-2,4-pentadienylidene cyanoacetyl)benzofuran, 1.5 g. (1 mol.) of 1,3-indandione, 20 cc. of pyridine and 1 g. (1 mol.) of triethylamine were mixed together and heated at steam bath temperature for 10 minutes. Dye separated from the chilled reaction mixture on treatment with excess of dilute hydrochloric acid. The crude, washed dye was purified in the usual manner and obtained as a black powder, M. P. 185-187°C., with decomposition.

## EXAMPLE 16



## [2-cyanoacetylbenzofuran] [3-phenyl-5 (4)-isoxazolone-(4)] pentamethineoxonol

3.8 g. (1 mol.) of 2-(5-acetanilido-2,4-pentadienylidene cyanoacetyl)benzofuran, 1.6 g. (1 mol.) of 3-phenyl-5(4)-isoxazolone, 30 cc. of pyridine and 1 g. (1 mol.) of triethylamine were mixed together and heated at steam bath temperature for 15 minutes. Dye separated from the reaction mixture on chilling and acidification with dilute hydrochloric acid. The crude, washed dye was purified in the usual manner. It was obtained as minute dark crystals, M. P. 191-193°C., with decomposition.

For the preparation of filter layers from 5 milligrams to 25 milligrams of dyes are wet with 2 cc. of triethylamine or pyridine and dissolved in 10-20 cc. of methanol, acetone or other water-soluble miscible solvent. The solution is added to 100 cc. of 3% to 6% aqueous gelatin solution at 40°C. After adjusting the pH to its optimum value, the dye solution is coated on the support which may already have other photographic layers.

The preparation of filter layers may be illustrated by the following examples.

The filter solutions are made up much as in the two following examples.

(1) A 20 mg. portion of [2-cyanoacetylbenzofuran] [3-methyl-1-p-sulphenyl-5-pyrazolone-(4)] trimethineoxonol is wet with 1 cc. of pyridine and dissolved in 20 cc. of methanol. This solution is added to 50 cc. of 10% aqueous gel containing 25 mg. of polyvinyl pyridine metho-p-toluene sulfonate. Water is added to bring the volume to 100 cc. (=5% gel) and the pH is adjusted to 5.7. The solution is then ready for coating on the support.

(2) A 12 mg. portion of [2-cyanoacetylbenzofuran] [1,3-di-β-methoxy ethylbarbituric acid-(5)] pentamethineoxonol is wet with 1 cc. of pyridine and dissolved in 20 cc. of methanol. This solution of dye is added to 50 cc. of 10% aqueous gel. Water is added to bring the volume to 100 cc. (=5% gel) and the pH is adjusted to 6.0. The solution is then ready for coating on the support.

In the accompanying drawing, the various figures are enlarged sectional views of photographic elements having filter layers or anti-halation layers made according to our invention. As shown in Fig. 1, a support 10 of any suitable ma-

terial such as cellulose nitrate, cellulose acetate, synthetic resinous material or opaque material such as paper is coated with an emulsion layer 11 and an overcoating layer 12 containing an unsymmetrical methine or polymethine oxonol dye according to our invention.

Fig. 2 illustrates a multi-layer photographic element for color photography in which the support 10 is coated with sensitive layers 13, 14 and 15 which record, respectively, the red, green and blue regions of the spectrum. Between the emulsion layers 14 and 15 there is a filter layer 16 containing a yellow methine or polymethine oxonol dye. This filter layer serves a purpose well known in color photography of preventing exposure of a lower layer of the element by light which the filter layer absorbs. The dye may also absorb light in other regions such as the ultraviolet region of the spectrum.

Fig. 3 represents a film having an anti-halation layer containing an oxonol dye according to our invention. As shown therein, the support 10 carries an emulsion layer 11 on one side and an anti-halation layer 18 containing an oxonol dye on the opposite side.

As stated above, the oxonol dyes are found to be useful in filter or anti-halation layers. The dyes in general are dissolved in water as the sodium, pyridinium or triethylamine salt, or in organic solvents such as alcohol or acetone and then dispersed in gelatin or other protein or synthetic vehicle such as polyvinyl alcohol.

The dyes used according to our invention have a number of advantages. They may contain acidic groups such as carboxylic acid or sulfonic acid groups and may therefore be mordanted by addition of equivalent amounts of cations such as  $Pb^{++}$ ,  $Ca^{++}$ ,  $Ba^{++}$ , etc., or organic agents such as polyvinyl pyridine metho-p-toluene sulfonate and other high molecular weight quaternary salts. Since the dyes are unsymmetrical, they may contain only a single acid group and are frequently easier to mordant than dyes containing two or more acid groups.

A further advantage of the unsymmetrical dyes is that they permit the choice of a wider range of spectral absorptions and thus give a better chance of meeting specific requirements of absorption maxima and distribution of absorption properties. The dyes are bleached in the usual photographic processing solutions such as developing and fixing solutions.

It will be understood that the examples included herein are illustrative only and that our invention is to be taken as limited only by the scope of the appended claims.

We claim:

1. A photographic element comprising a support having thereon at least one sensitive silver halide emulsion layer and a light-absorbing layer containing a dye having the formula:



where  $X$  represents the atoms necessary to complete a ring selected from the class consisting of barbituric acid, thiobarbituric acid, pyrazolone, oxindole, indandione and isoxazolone,  $Y$  represents a group selected from the class consisting of aryl groups of the benzene series and benzofuran, and  $n$  is a digit from 0 to 2.

2. A photographic element comprising a support having thereon at least one sensitive silver

11

halide emulsion layer and a light-absorbing layer containing a dye having the formula:



where **X** represents the atoms necessary to complete a barbituric acid ring, **Y** represents a benzofuran ring and *n* is a digit from 0 to 2.

3. A photographic element comprising a support having thereon at least one sensitive silver halide emulsion layer and a light-absorbing layer containing a dye having the formula:



where **X** represents the atoms necessary to complete a pyrazolone ring, **Y** represents a benzofuran group and *n* is a digit from 0 to 2.

4. A photographic element comprising a support having thereon at least one sensitive silver halide emulsion layer and a light-absorbing layer containing a dye having the formula:

5

12



10

where **X** represents the atoms necessary to complete a thiobarbituric acid ring, **Y** represents a benzofuran group and *n* is a digit from 0 to 2.

5. A photographic element comprising a support having thereon at least one sensitive silver halide emulsion layer and a light-absorbing layer containing [2-cyanoacetylbenzofuran] [3-methyl-1-p-sulfophenyl-5-pyrazolone (4)] trimethineoxonol.

15

GRAFTON H. KEYES.  
LESLIE G. S. BROOKER.

## REFERENCES CITED

20 The following references are of record in the file of this patent:

## UNITED STATES PATENTS

| Number    | Name   | Date         |
|-----------|--------|--------------|
| 2,186,608 | Keyes  | Jan. 9, 1940 |
| 2,274,782 | Gaspar | Mar. 3, 1942 |

25